

## UNITED STATES PATENT OFFICE

1,957,873

## WOOD PRESERVATIVE

Karl Heinrich Wolman, Berlin-Grunewald, and  
 Hans Pflug, Berlin-Wilmersdorf, Germany, as  
 signors to Grubenholzimpregnierung G. m. b.  
 H., Berlin, Germany

No Drawing. Application July 10, 1930, Serial  
 No. 467,130. In Germany August 10, 1929

3 Claims. (Cl. 134—78.6)

The present invention relates to improved water-soluble preservatives for wood. It is known, that numerous water-soluble preservatives, such as the salts of hydrofluoric acid and fluosilicic acid, or the soluble arsenic compounds, for instance the soluble salts of arsenic acid and arsénous acid, have a good fungicidal action, but in practice do not show a protective action, which is in all cases satisfactory and more especially 5 sufficiently durable, since they may easily be leached out of the wood upon water entering the wood in the form of atmospheric deposits, such as rain or snow or soil water or the like and thus become incapable of protecting the wood against 10 destructive fungi and pests. For the purpose of avoiding this drawback it has already been proposed, to use difficultly-soluble compounds for preserving wood. It has been proposed for instance to impregnate the wood successively with 15 two solutions, the ingredients of which react in the wood to form a difficultly-soluble, preservative compound. Use has also been made of solutions, which when they dry in the wood involve chemical changes between the constituents of the solution, which cause the formation of difficultly-soluble 20 compounds in the wood. Both processes possess, however, certain disadvantages. If two solutions are introduced into the wood, which by their reaction are to form the difficultly-soluble preservatives, there is always the difficulty that the 25 reaction of the two solutions is not complete, since the presence of the first solution introduced into the wood hinders the penetration of the second solution, more especially into the deeper layers 30 of the wood. The processes belonging to the second group mentioned above, in which therefore the wood is only treated with one solution, from which the difficultly-soluble preservative is 35 formed after drying, show the drawback that the 40 solutions are not sufficiently stable and readily decompose more especially at an increased temperature. If therefore such solutions are kept for some time, it may easily happen that the 45 composition of the solution changes in an undesirable way before impregnation, and the same position may arise if the solutions are heated prior to the 50 impregnation, which is desirable in many cases to facilitate impregnation.

We have found that these drawbacks can be 55 avoided and at the same time a preservation of the wood which is resistant to leaching out by water can be obtained, if other compounds such as for instance chromic acid or dichromic acid or salts of these acids, namely potassium chromate, sodium chromate, alkali dichromates,

potassium dichromate or sodium dichromate, also suitable compounds of the light and heavy metals singly or in mixture are added to the soluble protectives, for instance fluorine compounds, more especially the soluble salts of hydrofluoric acid or fluosilicic acid, arsenic compounds, for instance the soluble salts of arsenic acid and arsénous acid. These former substances are capable on the one hand of diminishing the capacity of the said soluble preservatives to be leached out, 60 and on the other hand of themselves becoming bound to the wood substance in such a way that they are difficult to wash out. These substances used as additions to the water-soluble preservatives we term in our application "fixatives". These 65 fixatives can be dissolved together with the protectives in water. After introduction into the wood or after the drying of the impregnating solution, the added substances effect a fixing of the 70 preserving media and also themselves become 75 fixed to the wood fibres in such a way that they are difficult to wash out. We use the fixatives in such quantities, that of the preserving agents introduced into the wood at least 30% are fixed 80 to the wood fibres so that they cannot be washed 85 out. We mean by this that the wood treated with the preservatives according to the invention can be treated with water at ordinary temperature without more than 70% of the preservative originally introduced into the wood being 90 able to be leached out. Preferably we employ the fixatives in amounts of more than 20% of the total amount of the salts. The composition of the preservative can naturally vary within wide 95 limits and depends upon the protective substances and the fixative used.

Other suitable fungicidal or insecticidal substances or substances reducing the inflammability of the wood, such as for instance nitrated phenols or their salts, phosphates, borates, acetates, salts 95 of ammonium and so on can also be added to the aforementioned mixtures of preservatives and fixative. Use may also be made of a mixture of several preservatives and a mixture of several fixatives.

The new preservatives can be used to impregnate wood in any suitable manner, for instance by saturating in closed vats with the use of vacuum and pressure, by steeping in the impregnating liquid in open troughs, by the so-called inoculation process, by introduction into receptacles, which are placed on or round the wood, by coating and the like. Prior to the impregnation there can be a suitable preliminary treatment of the wood, in which it is subjected for instance in a 110

manner known per se to a treatment with steam, electricity, air or gases. The aqueous solutions of the new impregnating media may also be used mixed with oily liquors, for instance as emulsions 5 or be used for so-called double impregnation, the wood being first saturated with the aqueous solution and then with an oily liquid or vice versa.

We will now give a few examples of the invention but stipulate that our invention is not limited either to the given substances or proportions 10 or measures.

*Example 1*

15 1 part of potassium bichromate and 1 part of sodium fluoride are mixed and a 2% aqueous solution prepared from this salt mixture. This solution is used to saturate wood in a closed vat according to the so-called full cell process at 70-80° C.

20 *Example 2*

45 parts of potassium bichromate, 50 parts sodium fluoride and 5 parts dinitrophenol are mixed and this salt mixture used in a manner known per se for impregnating wood in a 1.8% solution.

25 The excellent effect of the preservative according to the invention is evident for instance from the following: A salt mixture was prepared from 50% sodium fluoride, 45% potassium bichromate and 5% dinitrophenol. A 2% solution was prepared from the mixture and logs of sound, clean pinewood were fully saturated with the solution. In carrying out the saturation it was accurately determined how much solution or preservative 30 was introduced into the wood. After saturation the logs were dried by leaving them in the open air and when dry were cut up to the size of matches. The cut up wood was exposed to the leaching action of water at ordinary temperature. This 35 was done by shaking 100 grms. cut up wood in a glass flask of about 1-litre capacity with 600 ccms. water first for 2 hours, then with another 600 ccms. water for 4 hours and then with a further 600 ccms. water for 8 hours on a shaking machine.

40 45 The shaking with 600 ccms. water for 8 hours in each case was repeated five times more, so that in

all 8 shakings with 8×600 ccms. water took place in the whole 54 hours. A continued washing showed that further washing waters contained practically no more impregnating materials, so that the whole amount of impregnated salt, capable of being washed out was removed from the wood by the 8 shaking processes. The washing liquors were tested for their content of leached out constituents, and it was found that after the 8 shaking processes had been carried out, there 8 was still 36.5% of the preservative introduced into the wood, remaining therein.

9 The salts of the other light and heavy metals were tested in a similar way, but proved however in some cases less economical and in some cases 91 they gave less favourable results than the chromium salts.

What we claim is:

1. A water soluble preservative for wood fibre 95 consisting essentially of a water soluble salt of hydrofluoric acid to which a water soluble chromium salt is added as a fixative, the two being in about equal quantities so that more than 30% of the preservative will be fixed on the wood fibres and will not wash out.

100 2. A water soluble preservative for wood fibre consisting essentially of equal parts of a water soluble salt of hydro-fluoric acid and a water soluble salt of arsenic to which a water soluble salt of chromium has been added as a fixative in quantity 105 equal to about two-thirds of the amount of the preservative, so that more than 30% of the preservative will be fixed on the wood fibres and will not wash out.

110 3. A water soluble preservative for wood fibre consisting of about 40% of a water soluble salt of hydrofluoric acid, about 40% of water soluble arsenic salt and about 20% of dinitrophenol to which a water soluble chromium salt is added as a fixative in quantity equal to about three-fifths 115 of the amount of the preservative, so that more than 30% of the preservative will be fixed on the wood fibres and will not wash out.

KARL HEINRICH WOLMAN.  
HANS PFLUG.

120

50

125

55

130

60

135

65

140

70

145

75

150